

## UNITED STATES PATENT OFFICE

2,532,117

## NICKEL STEEL ALLOYS

Harold D. Newell, Beaver Falls, Pa., assignor to  
 The Babcock & Wilcox Tube Company, West  
 Mayfield, Pa., a corporation of Pennsylvania

No Drawing. Application September 17, 1946,  
 Serial No. 697,570

5 Claims. (CL. 75—125)

1

This invention relates to improved nickel alloy steel compositions and more particularly to nickel alloy steels resistant to certain corroding influences and having good toughness characteristics with ductility and resistance to impact at sub-zero temperatures.

Heretofore, it has been customary to use nickel steels for machine parts, for automotive parts, for carburized roller bearings and for other purposes in the usual form of SAE or NE grades with nickel contents up to 5% or thereabouts. Steels with up to this amount of nickel are also combined with small quantities of chromium, molybdenum, vanadium, silicon or other alloying ingredients, and the carbon content is adjusted to suit the end use or requirement for hardness, strength or other properties. High nickel steel alloys containing 30% or more nickel are also well known and have been used for their special properties of electrical resistance, low expansion rates or other features. Commercial steels, exclusive of stainless steels, have not been made and used containing more than about 5.25 per cent nickel and this is especially so of steels containing between about 7 per cent and 12 per cent nickel because such steels are hard and martensitic in character and lack ductility and are difficult to anneal so as to soften them for machining, expanding, bending or other forming operations. Consequently, such steels have previously not been available in tubing or pipe or other articles as they were considered to be laboratory curiosities not usable commercially because of their peculiar properties.

The present invention makes available nickel alloy steels of wide application in industry at costs substantially lower than those for the stainless steels now in commercial use. The nickel steel alloys in themselves are not considered stainless but nevertheless are much more corrosion-resistant than ordinary or low alloy steels in a variety of circumstances. The alloys may be made to possess remarkable physical properties or can be softened by heat treatment so as to be readily formed and used as hereinafter described. These steels can be used in welded constructions by the use of well-known welding methods if certain practices are followed as to preheating and postheating the metal following the welding operations.

The main object of the present invention is to provide a new series of nickel alloy steels which

2

may be varied as to composition to provide various properties of corrosion resistance to atmosphere, to alkaline solutions or mild organic acid conditions (pH 2.0 to 6.0), to chloride and sulphide solutions, or other forms of corrosion where presently available lower alloy content steels, including the commercial nickel steels, are not adequate or economical because of their lack of corrosion resistance or unsuitable physical properties for special fields of service. Another and more specific object is to provide for the manufacture of articles requiring steels having toughness and ductility such as tubes, pipe, rods, containers, valves and fittings, and other formed appurtenances for industrial use as in evaporators, exchangers, pipe lines, gas conversion equipment, equipment for liquified gases at low temperature and the like as are commonly used in the chemical, paper pulp, oil production and refining industries, and the like. A further object is to provide alloy steels having a new range of nickel contents for the manufacture of tubular products having exceptional toughness at sub-zero temperatures down to minus 320 F. below where ordinary and known steels of many kinds become exceedingly brittle and are hazardous in use.

The new series of nickel alloy steels made in accordance with the present invention have in general the following composition:

|                                                                                                                                                                                                                                                                                                                                                                                                                                  | Per cent                                             |
|----------------------------------------------------------------------------------------------------------------------------------------------------------------------------------------------------------------------------------------------------------------------------------------------------------------------------------------------------------------------------------------------------------------------------------|------------------------------------------------------|
| Carbon                                                                                                                                                                                                                                                                                                                                                                                                                           | 0.03 to 0.20                                         |
| Manganese                                                                                                                                                                                                                                                                                                                                                                                                                        | 0.20 to 1.00                                         |
| Silicon                                                                                                                                                                                                                                                                                                                                                                                                                          | 0.03 to 0.40                                         |
| 35 Nickel                                                                                                                                                                                                                                                                                                                                                                                                                        | 7.50 to 12.00                                        |
| Chromium                                                                                                                                                                                                                                                                                                                                                                                                                         | 0.02 to 6.00                                         |
| Copper                                                                                                                                                                                                                                                                                                                                                                                                                           | 0.05 to 2.00                                         |
| Molybdenum                                                                                                                                                                                                                                                                                                                                                                                                                       | 0.03 to 2.00                                         |
| 40 Titanium, columbium, zirconium or vanadium singly or in combination                                                                                                                                                                                                                                                                                                                                                           | 0.0 to 1.00 with the balance substantially all iron. |
| 45                                                                                                                                                                                                                                                                                                                                                                                                                               |                                                      |
| In making the alloys comprising this invention, it is preferable to follow good alloy steel making practice. The steels are best made in the electric arc furnace although induction furnaces or other processes may be employed. Sulphur content should be low because of the susceptibility of nickel steels to sulphur with attendant affect on rolling properties. Accordingly, fuels for heating purposes in the rolling of |                                                      |
| 50                                                                                                                                                                                                                                                                                                                                                                                                                               |                                                      |

ingots, blooms, bars or tubes should be low in sulphur for best results.

The steels should be thoroughly deoxidized, usually with one to two pounds or more of aluminum per ton to produce steels with fine grained characteristics having high toughness and ductility. This is necessary for retention of impact strength at low temperature and such thorough deoxidation has the further advantage of stimulating reaction rates during annealing and reducing strain-aging properties. Silicon is preferably kept below 0.25 per cent and the steels should be poured into hot-topped molds.

With respect to composition, the nickel content, although not limited thereto, is usually ranged between 8 and 10 per cent in a low carbon base, the carbon being restricted in most cases to 0.12 per cent maximum and, where maximum ductility and softness is required in the finished product, as in tubes for bending or expanding, the carbon should be under 0.10 per cent, i. e. about 0.06 to 0.09 per cent. Even lower carbon may be advantageous in certain circumstances to avoid formation of a hard martensite-like constituent which has heretofore been characteristic of alloy steels having a nickel content in the range disclosed. Copper is usually added to the composition for its beneficial effect in creating better corrosion resistance toward the atmosphere and other corrosive media including alkalies and mild acids. The usual addition is 0.20 to 0.40 per cent copper. Where high ultimate strengths are required the copper may be raised to 1.00 per cent or more and this adds further to the corrosion resistant properties of the alloys, at the same time permitting age-hardening reactions to occur in the steel upon tempering treatments, with decided improvement in physical properties. In fact, carbon can be kept very low in my alloy steels, and copper may be used to strengthen them by precipitation hardening on applying appropriate heat treatments. Such heat treatments consist of normalizing or quenching from above the  $A_3$  point and thereafter tempering between about 850 F and 1100 F.

Molybdenum may be added as required to the extent of upwards of 2.00 per cent to benefit physical properties and to considerably improve corrosion resistance particularly under mild acid corrosion conditions. When used, a preferred amount is approximately 0.50 per cent molybdenum.

Chromium, when added to my nickel steels, is used for improvement of corrosion resistance. It also alters physical properties. Approximately 5 per cent chromium may be added although a lesser amount has a beneficial effect. For resistance to alkalies or for good toughness at low temperature, chromium is not required and is not incorporated in my preferred alloy.

Manganese is incorporated as in good alloy steel practice and may be present between about 0.20 and 1.00 per cent. About 0.30/0.60 per cent is the usual addition. Phosphorus is generally low and for maximum softness, silicon can be ranged near the low limit or about 0.20-0.05 per cent.

The usual nickel alloy steels having a nickel content of about 5.0 to 12.0 per cent or more tend to be hard and brittle due to the characteristic formation of a martensite-like constituent which is difficult to break down to ferrite and carbides even on extended annealing cycles. When the alloying constituents previously described are combined in the proportions disclosed, and the

carbon is limited to .20 per cent maximum, or more often is restricted to .12 per cent or less, the hardenability of the steel is reduced and the working, annealing and machining of these nickel steels is greatly improved. However, to further reduce hardenability and to provide easy workability, good ductility and ease of annealing, such as necessary in the manufacture of ductile seamless tubes suitable for expanded joints or bends, I have found it desirable to incorporate one or more strong carbide formers to tie up carbon and render it ineffective in forming and retaining the hard and brittle martensite-like constituent. This is accomplished by adding titanium up to the equivalent of four or more times the carbon content. When columbium is added up to ten times the carbon content, it has an equal effect in suppressing hardenability. Zirconium and/or vanadium may also be used for their effects of this kind. For this purpose, zirconium may be added in a ratio up to 8-10 times the carbon content and vanadium up to 4 or more times the carbon content, depending on whether it is desired to fairly fully suppress or only partially suppress hardening reactions. These carbide forming elements may be used singly or together in any of many ratios to tie up carbon, with any combination of these several carbide formers incorporated in the steels up to a total of not exceeding 1.00 per cent construed as coming within the scope of the invention. The titanium, vanadium, columbium and/or zirconium may be added in the form of the usual ferro-alloys as metals, or special deoxidizers or reduced into the metal from their oxides or other compounds. Titanium is the preferred addition because of the low ratio required for carbide formation and because it is most economical. Other advantages accrue from using these carbide formers in my alloys as they tend to suppress caustic embrittlement and they reduce strain-aging effects in the metal.

As is disclosed, several variations of my alloy may be used depending upon exact use. My preferred range for general use is:

|               | Per cent   |
|---------------|------------|
| Carbon (max.) | 0.12       |
| Manganese     | 0.40- 0.60 |
| Nickel        | 8.00-10.00 |
| Silicon       | 0.05- 0.25 |
| Copper        | 0.20- 0.40 |

with the balance substantially all iron.

Typical heats of this nickel steel alloy made for use as tubes in alkali evaporators had analyses and grain sizes as follows:

Table I

| Heat No. | C    | Mn   | Si   | Cr   | Ni   | Cu   | Mo   | McQuaid-Ehn Grain Size |
|----------|------|------|------|------|------|------|------|------------------------|
| 1-----   | 0.06 | 0.47 | 0.18 | 0.11 | 8.96 | 0.35 | 0.05 | 6-7 (5)                |
| 2-----   | 0.09 | 0.41 | 0.20 | 0.04 | 9.12 | 0.23 | 0.04 | 6-7 (5)                |
| 3-----   | 0.07 | 0.46 | 0.24 | 0.03 | 8.94 | 0.36 | 0.04 | 6-7 (5)                |
| 4-----   | 0.07 | 0.44 | 0.18 | 0.09 | 9.04 | 0.39 | 0.04 | 6-7 (5)                |
| 5-----   | 0.06 | 0.47 | 0.22 | 0.10 | 8.96 | 0.30 | 0.07 | 6-7 (5)                |
| 6-----   | 0.07 | 0.47 | 0.17 | 0.03 | 8.80 | 0.37 | 0.06 | 6-7 (5)                |

The above steel, in the normalized condition, in specimens from 3 inch rounds, had impact strengths as recorded in Table II at room temperature and minus 320 F. On softening by tempering, after normalizing, the impact strengths improved greatly as may also be noted in the same table.

Table II.—Impact properties<sup>1</sup>

| Heat No. | Normalized at 1575 F. |         | Normalized, 1575 F.<br>Drawn, 1050 F. |         |
|----------|-----------------------|---------|---------------------------------------|---------|
|          | R. T.                 | -320 F. | R. T.                                 | -320 F. |
| 1.       | 36.0                  | 20.2    | 56.0                                  | 47.3    |
| 2.       | 38.0                  | 21.2    | 55.0                                  | 41.5    |
| 3.       | 40.0                  | 24.0    | 54.0                                  | 37.0    |
| 4.       | 35.0                  | 20.7    | 50.0                                  | 47.3    |
| 5.       | 35.0                  | 20.5    | 50.0                                  | 47.8    |
| 6.       | 35.0                  | 19.0    | 48.0                                  | 47.8    |

<sup>1</sup> Standard Charpy specimen .394" square-drilled keyhole notch. Values shown are average of three specimens of each heat at each temperature. All tests made on specimens taken longitudinal to rolling direction.

Other alloys coming within the scope of the invention are disclosed as to composition in Table III. Usual heat treatments applied consist of normalizing at about 1575 F., or double normalizing and tempering at about 1050 F. With selection of composition and treatment, a wide range of physical properties may be provided. Typical properties obtained on my alloys in these circumstances may be noted in Table IV. In surveying these values, it may be noted that titanium additions are useful for softening and reduction of silicon content is also helpful toward that end where maximum ductility might be required in the article.

The preferred double normalizing heat treatment consists in first normalizing at a temperature of approximately 1625 F. and a second normalizing at a temperature of approximately 1450 F.

Table III.—Chemical analysis

| Alloy | C    | Mn   | Si   | Ni   | Cu   | Mo   | V    | Ti   | Cr   |
|-------|------|------|------|------|------|------|------|------|------|
| 7.    | 0.12 | 0.95 | 0.15 | 8.61 | 0.06 |      |      |      | 0.50 |
| 8.    | 0.08 | 0.37 | 0.10 | 9.04 |      | 0.20 |      |      |      |
| 9.    | 0.09 | 0.30 | 0.22 | 9.93 | 0.65 |      |      |      |      |
| 10.   | 0.10 | 0.24 | 0.21 | 9.32 |      |      | 0.38 |      |      |
| 11.   | 0.07 | 0.24 | 0.20 | 9.21 |      |      |      | 0.22 |      |
| 12.   | 0.06 | 0.20 | 0.18 | 9.61 | 0.63 | 0.56 |      |      |      |
| 13.   | 0.08 | 0.45 | 0.20 | 9.56 | 0.61 | 0.58 |      |      | 5.50 |
| 14.   | 0.10 | 0.60 | 0.38 | 9.49 | 0.48 | 0.53 |      | 0.21 | 5.53 |
| 15.   | 0.06 | 0.27 | 0.09 | 9.09 | 0.48 | 0.50 |      |      |      |

Table IV.—Physical properties

|                    | Alloy | Condition                      | Ultimate,<br>p. s. i. | Yield,<br>p. s. i. | Elong.<br>Per Cent<br>in 2" | Red. of<br>Area,<br>Per Cent | BHN | Impact,<br>Ft. Lbs. |
|--------------------|-------|--------------------------------|-----------------------|--------------------|-----------------------------|------------------------------|-----|---------------------|
| .50 Cr.            | 7     | Normalized                     | 185,750               | 151,000            | 13.0                        | 47.2                         | 367 | 18.5                |
|                    |       | Double Normalized              | 191,200               | 159,250            | 11.5                        | 44.4                         | 408 | 18.5                |
| .20 Mo.            | 8     | Normalized                     | 133,250               | 117,750            | 20.0                        | 60.1                         | 285 | 32.5                |
|                    |       | Double Normalized and Tempered | 139,000               | 113,000            | 15.0                        | 55.5                         | 287 | 25.0                |
| .65 Cu.            | 9     | Normalized                     | 131,600               | 108,800            | 15.0                        | 49.9                         | 309 | 27.0                |
|                    |       | Double Normalized and Tempered | 120,750               | 109,150            | 20.0                        | 57.7                         | 265 | 36.5                |
| .38 V.             | 10    | Normalized                     | 147,600               | 125,100            | 15.5                        | 57.3                         | 305 |                     |
|                    |       | Double Normalized              | 130,500               | 110,500            | 17.0                        | 58.4                         | 278 | 25.0                |
| .22 Ti.            | 11    | Normalized                     | 106,300               | 96,250             | 22.0                        | 65.8                         | 230 | 41.0                |
|                    |       | Double Normalized and Tempered | 99,000                | 79,750             | 26.0                        | 68.2                         | 227 | 54.5                |
| .63 Cu.<br>.56 Mo. | 12    | Normalized                     | 142,400               | 118,900            | 15.0                        | 54.4                         | 307 | 22.0                |
|                    |       | Double Normalized              | 137,000               | 114,200            | 26.0                        | 45.8                         | 293 | 20.5                |
| .61 Cu.<br>.58 Mo. | 13    | Normalized                     | 133,000               | 122,500            | 18.0                        | 51.5                         | 300 | 33.0                |
|                    |       | Double Normalized and Tempered | 192,000               | 153,500            | 12.0                        | 47.0                         | 427 | 15.0                |
| .55 Cr.<br>.48 Cu. | 14    | Normalized                     | 152,250               | 142,000            | 18.0                        | 59.4                         | 342 | 21.5                |
|                    |       | Double Normalized              | 187,000               | 158,000            | 13.5                        | 50.8                         | 391 |                     |
| .53 Mo.<br>.21 Ti. | 15    | Normalized                     | 202,500               | 154,300            | 12.5                        | 44.2                         | 385 | 26.5                |
|                    |       | Double Normalized and Tempered | 167,200               | 165,500            | 13.0                        | 51.2                         | 363 | 43.0                |
| .48 Cu.<br>.50 Mo. | 15    | Normalized                     | 144,000               | 119,750            | 15.0                        | 53.3                         | 312 | 18.0                |
|                    |       | Double Normalized              | 138,800               | 119,300            | 17.0                        | 58.9                         | 299 | 21.5                |
|                    |       | Double Normalized and Tempered | 137,000               | 124,800            | 21.0                        | 61.2                         | 303 | 31.5                |

Using the compositions set forth, I am able to provide corrosion resistance in a variety of media which exceeds that available in the usual structural nickel steels, particular advantage being secured when articles of my alloys are exposed to alkaline media. Good resistance is also secured under mildly acidic conditions. Physical properties may be altered in my steels by variation within the range of composition set forth to obtain high strength with reasonable ductility, or softer more ductile material may be provided as required. My preferred alloy composition offers high impact strength and retains its toughness to much lower temperatures than any of the lesser alloy content engineering steels and consequently may be employed to replace stainless austenitic steels or non-ferrous metals in equipment intended for sub-zero service. It is especially useful when service temperatures fall below about minus 175 F.

My alloys may be rolled or manufactured into useful industrial articles such as tubing and pipe for conveying fluids, into sucker rods, valve parts, oil well appurtenances, bearings for carburizing and into other articles as desired. Ordinary equipment usually available in steel mills may be used to convert the metal from ingot to other wrought forms. My alloy steels can be substituted for steels having lesser corrosion resistance or inferior physical properties at moderate increase in cost over those presently available commercially and at much lower cost than for the high chromium-nickel stainless steels.

The analyses given in Table III are illustrative and the objects of the present invention may be realized by altering the composition within the ranges set forth in the claims made hereinafter.

I claim:

1. A forgeable and machinable alloy steel characterized by high resistance to alkali and mild acidic corrosion, said steel having the following composition
  - from 0.03 to 0.20% carbon
  - from 0.20 to 1.00% manganese
  - from 0.02 to 0.40% silicon
  - from 7.50 to 12.00% nickel
  - from 0.20 to 2.00% copper

up to 6.00% chromium  
up to 2.00% molybdenum

and up to 1.00% of a carbide former selected from the group consisting of titanium, columbium, zirconium and vanadium; balance iron and incidental impurities.

2. A forgeable and machinable alloy steel characterized by high resistance to alkali and mild acidic corrosion, said steel having the following composition

up to 0.12% carbon  
from 0.40 to 0.60% manganese  
from 8.00 to 10.00% nickel  
from 0.05 to 0.25% silicon  
from 0.20 to 2.00% copper

balance iron and incidental impurities.

3. A forgeable and machinable alloy steel characterized by high resistance to alkali and mild acidic corrosion, said steel having the following composition

from 0.06 to 0.09% carbon  
from 0.40 to 0.50% manganese  
from 8.80 to 9.20% nickel  
from 0.15 to 0.25% silicon  
from 0.20 to 0.40% copper  
from 0.03 to 0.11% chromium  
from 0.04 to 0.07% molybdenum

balance iron and incidental impurities.

4. A forgeable and machinable alloy steel characterized by high resistance to alkali and mild

acidic corrosion, said steel having the following composition

up to 0.12% carbon  
from 0.30 to 0.60% manganese  
from 8.00 to 10.00% nickel  
up to 0.25% silicon  
from 0.20 to 0.40% copper  
up to 0.50% molybdenum

10 and titanium up to 4 times the carbon content; balance iron and incidental impurities.

5. A nickel steel alloy tubular article composed of the alloy steel defined in claim 1; said article having been normalized and tempered.

15

HAROLD D. NEWELL

#### REFERENCES CITED

The following references are of record in the file of this patent:

20

#### UNITED STATES PATENTS

| Number    | Name           | Date           |
|-----------|----------------|----------------|
| 1,317,593 | Richardson     | Sept. 30, 1919 |
| 1,341,992 | McClure        | June 1, 1920   |
| 2,191,790 | Becket         | Feb. 27, 1940  |
| 2,194,178 | Becket et al.  | Mar. 19, 1940  |
| 2,206,370 | Scherer        | July 2, 1940   |
| 2,281,219 | Ziegler et al. | Apr. 28, 1942  |

#### FOREIGN PATENTS

| Number  | Country | Date          |
|---------|---------|---------------|
| 743,179 | France  | Mar. 25, 1933 |